

# UNITED STATES PATENT OFFICE.

WILLIAM N. BLAKEMAN, JR., OF MOUNT VERNON, NEW YORK.

## PAINT VEHICLE.

1,423,389.

Specification of Letters Patent. Patented July 18, 1922.

No Drawing.

Application filed April 16, 1921. Serial No. 461,961.

To all whom it may concern:

Be it known that I, WILLIAM N. BLAKEMAN, Jr., a citizen of the United States, and resident of the city of Mount Vernon, in the 5 county of Westchester and State of New York, have invented a new and useful Paint Vehicle, which invention is fully set forth in the following specification.

The object of this invention is to produce 10 a vehicle which, when combined with a pigment, will show an increased resistance to weathering attacks and cause the paint to approach more nearly to a permanent covering.

15 The present system of structural painting is largely based upon the unique union of Dutch white lead as a pigment and linseed oil as a vehicle. These, when properly ground together, form a hydrated metallic 20 soap, which, when spread on a plain surface, furnishes a smooth and homogeneous insoluble film. The atmospheric elements, however, soon attack the bond, which is the oil-vehicle, in this combination, and cause it 25 to pass by insensible gradations from an insoluble to a soluble condition, relaxing the bonding effect, releasing the pigment, and thus rapidly disintegrating the paint. This 30 early destruction of the present paint films, by atmospheric hydrolysis, aided by a weak alkaline reaction of the Dutch white lead pigment, is owing to the yielding character of linseed oil to weak hydrolytic influences; as, being strong in its oxygen affinities, it is 35 feeble in its resistance to even weak atmospheric hydrolytic action, becoming progressively sensitive to incipient hydrolysis by its progressive oxidation.

I have discovered that this disintegration 40 of all oil paint films can be delayed very greatly in its inception, and its progressive development indefinitely retarded, by reinforcing and fortifying the oil-vehicle employed, with non-drying oils or fats which 45 show a resistance to feeble saponifying attack or a repellent indifference to incipient atmospheric hydrolysis, so that, such non-drying oils will enter into combination with any drying-oil-vehicle, or drying-oil paint- 50 compound.

The non-drying oils which may be used are preferably those belonging to the group of vegetable fatty oils, and of these I prefer cocoanut oil and palm-kernel oil (or palm- 55 nut oil), both of which have a high resistance to weak hydrolytic action. These sub-

stances, which are flowing oils at summer heats, but chill to a solid or semi-solid condition at somewhat lower temperatures, are miscible with and soluble in oil-vehicles by 60 the aid of heat and can be introduced to the extent of from 5% to 20%, and will not cloud, flock, or chill out, but will remain in clear solution at temperatures very much below their thickening point. The result 65 will be a great improvement in the spreading power of the vehicle for all pigments, particularly anhydrous pigments, and especially when the vehicle carries an appreciable proportion of mineral oil, such as a 70 mineral oil of the Texas oil type.

Because of its abundance on the market, I prefer to use cocoanut oil, and if five or six parts of linseed oil, carrying 10% of cocoanut oil, be ground with twelve parts of 75 Dutch white lead, and spread on a plain surface, the mixture will firm to the touch in eight or nine hours, under favorable atmospheric conditions, and subsequently indurate into a durable film, the resistance of 80 the film to the elements being strongly supported by the presence of the cocoanut oil and the life of the paint greatly prolonged.

I have further discovered that tung oil 85 is a very efficient solvent for these non-drying oils or fats, even at common temperatures, and, when added in the proportion of from 12% to 15% to the oil-vehicle, prevents clouding or flocking at temperatures approaching freezing, and reduces the firm- 90 ing of the paint to one third or one half the time—thus: if five or six parts of linseed oil, carrying 10% of cocoanut oil and 15% of tung oil, be ground with twelve parts of Dutch white lead, and spread on a plain 95 surface, the mixture will firm to the touch in from two and one-half to three hours, under favorable atmospheric conditions, and subsequently indurate into a permanent film resistant to atmospheric and abrasive influences. A mixture of six parts of cottonseed oil, carrying 15% of tung oil and 10% of cocoanut oil, and ten parts of zinc lead (composed of 60% zinc oxide and 40% lead sulphate) will firm to the touch in four or 100 five hours under like atmospheric conditions.

Very satisfactory compositions can be formed, especially with anhydrous pigments, by using in the vehicle a proportion of a 110 mineral oil of the Texas type, either in an untreated condition, or hydrogenated or

oxidized or both; or a mineral oil of the Pennsylvania type hydrogenated or oxidized, or both. I prefer oxidized Texas oil. Thus, if six parts of cottonseed oil carrying 5% of cocoanut oil, 15% of tung oil and 10% of oxidized Texas oil, be ground with ten parts of zinc lead, the mixture when spread will firm and indurate satisfactorily and form an economical and permanent paint.

10 With slight changes in proportions of vehicles and pigments, all the oils (drying, semi-drying, non-drying, and mineral) and all the pigments (hydrated and anhydrous) which fall within the economical scope of 15 the painting art, can be employed.

In all cases, the usual proportion of a suitable commercial drier is to be used.

Light, heat, electricity, agitation, pressure, 20 oxidation and hydrogenation, may be employed if deemed advisable.

It will, of course, be understood that by the term "oil", as used in this specification and in the claims, to designate the vegetable non-drying oils and fats which have a high 25 resistance to hydrolysis, I intend to cover the use of such substances whether they are in a liquid, semi-solid, or solid, condition at the time of use.

The mixture of non-drying vegetable fatty oils, having a high resistance to hydrolysis, with tung oil, is broadly claimed in my application No. 505,626 filed October 5, 1921; the use of such non-drying fatty oils in paint-compositions is claimed in application No. 505,624, filed October 5, 1921; 35 and the grinding of pigments to paste form, in such non-drying fatty oils, is specifically claimed in application, No. 505,625 filed October 5, 1921.

Having thus fully described my invention, I claim:

1. A paint-vehicle carrying a non-drying vegetable fatty oil of high resistance to hydrolysis.
2. A paint-vehicle carrying cocoanut oil.
3. A paint-vehicle carrying a non-drying vegetable fatty oil of high resistance to hydrolysis and tung oil.
4. A paint-vehicle carrying cocoanut oil and tung oil.
5. A paint-vehicle carrying a non-drying vegetable fatty oil of high resistance to hydrolysis; tung oil; and a mineral oil.
6. A paint-vehicle carrying cocoanut oil; tung oil; and a mineral oil.

WM. N. BLAKEMAN JR.